# EUROPEAN PATENT SPECIFICATION

(11) **EP 2 990 499 B1**
(45) Date of publication and mention of the grant of the patent: **18.07.2018**
(21) Application number: 14788178.3
(22) Date of filing: 23.04.2014
(51) Int. Cl.: C22C 38/00, B21B 3/00, C21D 8/06, C22C 38/32, C22C 38/02, C22C 38/04, C22C 38/06, C22C 38/12, C22C 38/14, C22C 38/24, C22C 38/28, C21D 1/613, C21D 9/52, C21D 9/00

(54) **WIRE ROD AND METHOD FOR MANUFACTURING SAME**
WALZDRAHT UND VERFAHREN ZUR HERSTELLUNG DAVON
FIL MACHINE ET SON PROCÉDÉ DE FABRICATION

(30) Priority: 25.04.2013 JP 2013092775; 25.04.2013 JP 2013092782
(43) Date of publication of application: 02.03.2016
(73) Proprietor: Nippon Steel & Sumitomo Metal Corporation, Tokyo 100-8071 (JP)
(72) Inventor: OOBA Hiroshi, Tokyo 100-8071 (JP); ISO Arata, Tokyo 100-8071 (JP); TADA Tatsusei, Tokyo 100-8071 (JP); MANABE Toshiyuki, Tokyo 100-8071 (JP)
(74) Representative: Vossius & Partner Patentanwälte Rechtsanwälte mbB
(86) International application number: PCT/JP2014/061460
(87) International publication number: WO 2014/175345

(56) References cited:
- EP-A1- 2 175 043
- JP-A- 2000 192 148
- JP-A- 2008 007 856
- JP-A- 2010 229 469
- KR-A- 20130 034 029
- US-A1- 2009 223 610
- Naoya Kamikawa ET AL: "Effect of Deformation Temperature on Microstructure Evolution in ARB Processed Ultralow Carbon IF Steel", MATERIALS TRANSACTIONS, vol. 53, no. 1 25 December 2011 (2011-12-25), pages 30-37, XP055320678, Sendai DOI: 10.2320/matertrans.MD201115 Retrieved from the Internet: URL:https://www.jim.or.jp/journal/e/pdf3/5 3/01/30.pdf [retrieved on 2016-11-17]

## Description

### [Technical Field]

The present invention relates to a wire rod which is raw material of PC steel stranded wire for reinforcing a PC structure used for LNG (Liquefied Natural Gas) Tank of energy relating facility, and which has excellent low-temperature elongation and low-temperature toughness.

Priority is claimed on Japanese Patent Application No. 2013-092782, filed on April 25, 2013 and on Japanese Patent Application No. 2013-092775, filed on April 25, 2013, the content of which is incorporated herein by reference.

### [Related Art]

LNG tank is categorized as ground type and underground type. The present invention relates to a wire rod for ground type LNG tank and method for manufacturing the same. As the conventional art of the ground type LNG tank, Patent document 1 proposes metal double shell type LNG tank including a metal inner tank and a metal outer tank.

Generally, in the metal double shell type LNG tank, refrigerant is filled with clearance between the inner tank and the outer tank to limit increases in the temperature in the LNG tank and vaporization of LNG associated therewith. However, the structure includes the possibility of causing damage such as outflow of a lot of LNG, if a defect occurs at both of the inner tank and the outer tank. Therefore, in recent years, in order to further enhance safety, a technique in which a PC dike including PC structure (Prestressed Concrete Structure) is deployed outside the LNG tank and the inside of the PC dike is combined with the conventional metal double shell type LNG tank appears.

The PC dike in the technique includes concrete forming circular dike enclosing the LNG tank and PC steel stranded wire embedded in the concrete. Prestress is provided to the PC dike by tensioning the concrete along circumferential direction using the PC steel stranded wire. If LNG outflows from the LNG tank inside the PC dike, although tensile stress is applied to the PC dike along the circumferential direction thereof by the fluid pressure of the outflowing LNG, the prestress provided to the PC dike relieves the tensile strength. Patent document 2 (KR20130034029A) discloses a steel wire rod which has higher strength and better ductility than those of the conventional one without adding expensive elements, specifically a tensile strength of 1200 MPa or more and reduction of area of 45% or more, and a method of producing the same.

Patent document 3 (EP2175043 A1) discloses a steel rod superior in ductility for producing a steel wire suitable for steel cord, sawing wire, and other applications, and a method of producing the steel rod with high productivity and good yield in low cost.

### [Prior Art Document]

### [Patent Document]

[Patent Document 1] Japanese Unexamined Patent Application, First Publication No. 2006-234137

### [Disclosure of the Invention]

### [Problems to be Solved by the Invention]

On the other hand, the PC dike is continuously in a low-temperature state since heat is drawn by the LNG in the LNG tank. In addition, if outflow of LNG occurs as described above, LNG having temperature of -162°C or lower contacts with the concrete, and thus, the temperature around the PC steel stranded wire reinforcing the PC dike at the inner portion of the concrete may be greatly reduced. If low-temperature elongation and low-temperature toughness of the PC steel stranded wire are not sufficiently high, the PC steel stranded wire may break and the PC dike may fracture. Therefore, a wire rod which has better low-temperature elongation and better low-temperature toughness than the conventional wire rod for the PC steel stranded wire is needed. An object of the present invention is to provide a wire rod which has more excellent low-temperature elongation and more excellent low-temperature toughness than the conventional wire rod for the PC steel stranded wire in order to meet the needs of the markets.

### [Means for solving the Problem]

The inventors performed factual survey of use environment of the PC dike in order to enhance the tension providing effect in the PC dike constructing the PC type LNG tank (LNG tank including PC dike). As a result, in the actual use environment, it was found that there were cases in which the wire rod was exposed to an environmental temperature of about -40°C by heat transfer to the LNG in the LNG tank.

Therefore, various examinations with regard to a method for obtaining a wire rod having higher low-temperature elongation and higher low-temperature toughness as compared with the conventional PC steel stranded wire was performed. Specifically, in order to consider about the low-temperature elongation at first, a tensile test piece having especial shape shown in Figure 3 was manufactured from the wire rod and tensile test was performed with the tensile test piece. In addition, in order to consider about the low-temperature toughness, a 5mm subsize charpy impact test piece defined in JIS Z 2202 was manufactured from the wire rod and 2mm U-notch test was performed to the test piece to examine a relationship between the aspect of fracture surface and the charpy absorbed energy obtained by the test. As a result of the tests, it was found that the average grain size of pearlite block of the wire rod and a number density of coarse pearlite block affected to the low-temperature elongation at -40°C and fracture facet, which improve the low-temperature elongation and the low-temperature toughness.

Moreover, it was found that it was possible to provide the wire rod which had more excellent low-temperature elongation and more excellent low-temperature toughness as compared with the conventional wire rod for the PC steel stranded wire rod based on the above-described findings.

That is, the gist of the present invention of which the object is to solve the above-described problems is as follows.
(1) In a wire rod according to one embodiment of the present invention, the chemical composition consists of, in terms of mass%: C :0.60 to 1.20%; Si:0.80 to 1.30%; Mn:0.30 to 0.90%; P :0.020% or less; S :0.020% or less; N :0.0025 to 0.0060%; Cr:0 to 1.00%; V:0 to 0.800%; one or more selected from the group consisting of Al:0.005 to 0.100%, Ti:0.003 to 0.050%, and B :0.0005 to 0.0040%; and the remainder including Fe and impurity, wherein an average value of a grain size of a pearlite block in a cross section perpendicular to a wire rod axial direction is 23µm or less, and wherein a number density of the pearlite blocks having 40µm or more of the grain size in the cross section perpendicular to the wire rod axial direction is 0 to 20 pieces/mm².
(2) In the wire rod according to (1), the chemical composition may include one or more selected from the group consisting of, in terms of mass%:Cr: 0.10 to 1.00%, and V: 0.005 to 0.800%.
(3) In the wire rod according to (1), the chemical composition may include, in terms of mass%: C: 0.70 to 0.90%; Mn: 0.60 to 0.90%; and V: 0 to 0.500%.
(4) In the wire rod according to (3), the chemical composition may include one or more selected from the group consisting of, in terms of mass%: Cr: 0.50 to 1.00%, and V: 0.300 to 0.500%.
   In the wire rod according to any one of (1) to (4), wherein the chemical composition includes one or more selected from the group consisting of, in terms of mass%, Al: 0.020 to 0.050%, and Ti: 0.020 to 0.040%.
(6) A method for manufacturing the wire rod according to the other embodiment of the present invention, comprising: heating a steel piece having the chemical composition according to claim 3 or 4 to a rough-rolling temperature of 950 to 1040°C and rough-rolling; finish-wire-rolling at a finish-rolling temperature of 750 to 950°C; then, coiling at a coiling temperature of 730 to 840°C; and thereafter, air blast cooling to a temperature range of 5 to 35°C with a cooling rate of 15°C/sec or more, wherein the finish-rolling temperature and a strain rate in the finish-wire-rolling satisfy an expression A,
   13.7 ≤ log₁₀ {(dε / dt) × exp(63800 / (1.98 × (T + 273.15))} ≤ 16.5 :expression A, and
   wherein dε / dt expresses the strain rate in the finish-wire-rolling in terms of s⁻¹ and T expresses the finish-rolling temperature in terms of °C.

### [Advantageous Effects of Invention]

According to the above-described embodiments of the present invention, a wire rod for PC steel stranded wire which is favorable to usage as tendon of PC dike of PC-type LNG tank and which has more excellent elongation and toughness at about -40°C as compared with the conventional material can be provided by reducing the grain size of pearlite block and limiting the number density of coarse pearlite block.

### [Brief Description of Drawings]

Figure 1 is a graph indicating a relationship between an average grain size of pearlite block of the wire rod and reduction of area of the wire rod.
Figure 2 is a graph indicating a relationship between Z value in manufacturing the wire rod and the grain size of the pearlite block of the wire rod.
Figure 3 indicates a shape of low temperature tensile test piece.
Figure 4 indicates a collection position of 5mm subsize charpy impact test piece defined in JIS Z 2202.
Figure 5A indicates a grain size of the pearlite block of the example manufactured with a stelmor method.
Figure 5B indicates the grain size of the pearlite block of the comparative example.
Figure 6 indicates elongation of an example (No. 6) and a comparative example (No. 17) at -40°C.
Figure 7A indicates a grain size of the pearlite block of the example manufactured with DLP method.
Figure 7B indicates a grain size of the pearlite block of the comparative example.
Figure 8 indicates a relationship between pearlite block size (µm) and an absorbed energy (Charpy impact value) (J).
Figure 9A is a photograph indicating an observation result of a fracture surface of the impact test piece of the example with SEM.
Figure 9B is a photograph indicating an observation result of a fracture surface of the impact test piece of the comparative example with SEM.
Figure 10 is a flow chart indicating an example of a method for manufacturing the wire rod with a stelmor method.

### [Description of Embodiments]

In a wire rod for PC steel stranded wire according to the present embodiment (hereinafter "a wire rod according to the present embodiment") having excellent low-temperature elongation and low-temperature toughness, a chemical composition includes, in terms of mass%: C :0.60 to 1.20%; Si:0.30 to 1.30%; Mn:0.30 to 0.90%; P :0.020% or less; S :0.020% or less; N :0.0025 to 0.0060%; Cr:0 to 1.00%; V :0 to 0.800%; one or more selected from the group consisting of Al:0.005 to 0.100%, Ti:0.003 to 0.050%, and B :0.0005 to 0.0040%; and remainder including Fe and impurity, wherein an average value of a grain size of a pearlite block is 23µm or less in a cross section perpendicular to a wire rod axial direction, and wherein the number density of the pearlite block having 40µm or more of the grain size is 0 to 20 pieces/mm² in the cross section perpendicular to the wire rod axial direction.

At first, a reason for limiting the chemical composition of the wire rod according to the present embodiment will be described. Hereinafter, "%" expresses "mass%".

### (C: 0.60 to 1.20%)

C is an element having an effect of increasing a cementite ratio in the wire rod to increase strength of the wire rod. A lamellar spacing of the pearlite can be controlled by adjusting a patenting condition, and the strength of the wire rod can be increased by working. On the other hand, if an amount of C is less than 0.60%, a strength which can sufficiently tension a PC dike of a PC-type LNG tank cannot be obtained even if the above-described adjusting the patenting condition is performed.

If the amount of C in the wire rod is more than 1.20%, a mesh-shaped cementite forms in a structure in the wire rod. The mesh-shaped cementite may frequently cause breaking during wire drawing and may interfere production activity of the wire rod.

As a method for manufacturing the wire rod according to the present embodiment, both of DLP (Direct in-Line Patenting) method and stelmor method can be employed as follows. If the wire rod is manufactured with the stelmor method, it is preferable that the amount of C be 0.70 to 0.90%. If the wire rod is manufactured with the stelmor method, a cooling rate of the wire rod is lower than that in the manufacturing with the DLP method, and thus, the elongation and the toughness of the wire rod is relatively low. In order to compensate for the decrease in the strength, it is preferable that the lower limit of the amount of C be 0.70%. In addition, if the amount of C excessively increases, a pro-eutectoid cementite forms in the mesh shape at a grain boundary of prior austenite during cooling the wire rod, since the wire rod becomes a hyper-eutectoid steel (a steel having a structure containing both of pearlite and cementite). The mesh-shaped pro-eutectoid cementite significantly deteriorates the drawability of the wire rod. In order to prevent the mesh-shaped pro - eutectoid cementite from forming, it is preferable that the upper limit of the amount of C be 0.90%. It is more preferable that the amount of C be 0.80 to 0.90%.

### (Si: 0.30 to 1.30%)

Si is an element which acts as a deoxidizing element during refining. When 0.30% or more of Si is included, the deoxidizing effect is sufficiently expressed. Therefore, the lower limit of the amount of Si of the wire rod according to the present embodiment is 0.30%. Si also includes an effect for enhancing the strength of the wire rod. When 0.80% or more of Si is included, the effect of enhancing the strength is expressed. Therefore, the lower limit of the amount of Si of the wire rod according to the present embodiment may be 0.80%. In addition, although Si solid-solute strengthen ferrite, Si has an effect for rising a nose of isothermal transformation during heat treatment. Therefore, an excessive amount of Si increases cost for the heat treatment. Accordingly, in view of a capacity of the manufacturing equipments, the upper limit of the amount of Si is 1.30%.

As the method for manufacturing the wire rod according to the present embodiment, both of the DLP method and the stelmor method can be employed. If the wire rod is manufactured with the stelmor method, it is preferable that the amount of Si be 0.80 to 1.30%. If the wire rod is manufactured with the stelmor method, a cooling rate of the wire rod is lower than that in the manufacturing with the DLP method, and thus, the elongation and the toughness of the wire rod is relatively low. In order to compensate the decreasing of the strength, it is preferable that the lower limit of the amount of Si be 0.80%. It is more preferable that the amount of Si be 0.90 to 1.25%.

### (Mn: 0.30 to 0.90%)

Mn is an solid-solute strengthening element and has an effect of enhancing elongation and toughness of the wire rod and an effect of enhancing hardenability. In order to secure elongation and toughness of the wire rod, it is necessary that 0.30% or more of Mn be included. In addition, in order to further enhance the elongation of the wire rod, the lower limit of the amount of Mn may be 0.60%. On the other hand, if the amount of Mn is higher than 0.90%, a delay of transformation occurs in a center portion of the wire rod to cause a formation of micro martensite at a portion of untransformed austenite during manufacturing the wire rod. The micro martensite at the center portion of the wire rod causes breaking during drawing of the wire rod. Therefore, it is necessary that the upper limit of the amount of Mn is 0.90%.

As the method for manufacturing the wire rod according to the present embodiment, both of the DLP method and the stelmor method can be employed. If the wire rod is manufactured with the stelmor method, it is preferable that the amount of Mn be 0.60 to 0.90%. If the wire rod is manufactured with the stelmor method, the cooling rate of the wire rod is lower than that in the manufacturing with the DLP method, and thus, the elongation and the toughness of the wire rod is relatively low. In order to compensate the decreasing of the strength, it is preferable that the lower limit of the amount of Mn be 0.60%. It is more preferable that the amount of Mn be 0.70 to 0.90%.

### (P: 0.020% or lower)

### (S: 0.020% or lower)

P has an effect of embrittling the steel. Therefore, it is necessary that an upper limit an amount of P is 0.020%. When the wire rod is further securely prevented from low-temperature embrittlement, the upper limit of the amount of P may be 0.010%, 0.005%, or 0.001%.

S is an element which combines with Mn in the wire rod to form MnS. Since S segregates at a center portion of the steel during refining and solidifying the steel, MnS accumulates at the center portion of the steel. MnS deteriorates the low-temperature elongation of the steel. If an amount of S is more than 0.020%, the low-temperature elongation significantly deteriorates, and thus, the amount of S is 0.020% or lower. When the wire rod is further securely prevented from the low-temperature embrittlement, the upper limit of the amount of S may be 0.010%, 0.005%, or 0.001%.

In the wire rod according to the present embodiment, the lower the amount of P and the amount of S are, the better it is. Therefore, both of the lower limit of the amount of P and the lower limit of the amount of S is 0%.

### (N: 0.0025 to 0.0060%)

N is an element which combines with Al, Ti, and B to form nitrides. The nitrides act as a nucleuses of precipitation of the austenite, and thus, the grain size of the austenite can be controlled during heating the steel by controlling the number of the nitrides. If the amount of the nitrides increase, the grain is refined. If the amount of N is less than 0.0025%, the nitrides do not sufficiently form and the effect of refining the grain size cannot be sufficiently obtained. On the other hand, If the amount of N is more than 0.0060%, free N, which does not combine with Al, Ti, and B, become excess. The excess amount of free N causes age hardening to deteriorate the elongation and the toughness of the wire rod. Therefore, it is necessary that the amount of N be 0.0025 to 0.0060%. It is preferable that the amount of N be 0.0025 to 0.0040%.

In addition to the above-described elements, the wire rod according to the present embodiment further includes one or more selected from the group consisting of Al: 0.005 to 0.100%, Ti: 0.003 to 0.050%, and B: 0.0005 to 0.0040%.

### (Al: 0.005 to 0.100%)

Al acts as a deoxidizing agent during refining the steel. In addition, since Al forms composition with N in the steel, Al has an effect of fixing N. Due to fixing N, the steel can be prevented from age hardening. Furthermore, when B is included together with Al, due to fixing N, the amount of solute B can be increased.

However, if an amount of Al is less than 0.005%, the effect of fixing N by Al cannot be sufficiently obtained. On the other hand, if the amount of Al is more than 0.100%, Al₂O₃, which is formed by Al combining with oxygen in the steel, forms clusters. The clusters act as origins of cracking during drawing. Therefore, the amount of Al may be 0.005 to 0.100%. It is preferable that the amount of Al be 0.020 to 0.050%.

### (Ti: 0.003 to 0.050%)

Ti acts as the deoxidizing agent of the steel, similar to Al. In addition, since Ti forms chemical compound with N in the steel, Ti has an effect of fixing N. Due to fixing N, the steel can be prevented from age hardening. Furthermore, when B is included together with Ti, due to fixing N, the amount of solute B can be increased.

However, if the amount of Ti is less than 0.003%, the effect of fixing N by Ti cannot be sufficiently obtained. On the other hand, if the amount of Ti is more than 0.050%, TiC, which is formed by Ti combining with carbon in the steel, increase. TiC act as an origins of cracking during drawing. Therefore, the amount of Ti may be 0.003 to 0.050%. It is preferable that the amount of Ti be 0.020 to 0.040%.

As described above, Al and Ti have similar effects. Therefore, the amount of Al can be decreased by including Ti. In this case, a similar effect can be obtained.

### (B: 0.0005 to 0.0040%)

When B exists as the solute B in the austenite, B has an effect of enhancing the hardenability of the wire rod. If the amount of B is less than 0.0005%, the effect of enhancing the hardenability cannot be sufficiently obtained. On the other hand, if the amount of B is more than 0.0040%, B forms chemical compound with Fe and C to form a precipitates such as Fe₂₃ (C, B)₆, and the like. The precipitates act as the origins of cracking during drawing. Therefore, the amount of B may be 0.0005 to 0.0040%. It is preferable that the amount of B be 0.0009% to 0.0030%.

In addition to the above-described elements, the wire rod according to the present embodiment may further include, in terms of mass%, Cr: 0 to 1.00% or V: 0 to 0.800%.

### (Cr: 0 to 1.00%)

In the wire rod according to the present embodiment, it is not necessary to include Cr. Therefore, a lower limit of an amount of Cr is 0%. However, Cr has an effect of reducing lamellar spacing of the pearlite to enhance the strength of the wire rod. Due to the effect, the degree of increasing of the strength of the wire rod during drawing is enhanced. The effect is obtained in a case in which the amount of Cr is 0.10% or more, and thus, it is preferable that the amount of Cr be 0.10% or more. In addition, when the strength is further enhanced, it is preferable that 0.50% or more of Cr be included. If the amount of Cr is more than 1.00%, a termination time of pearlite transformation becomes long, and thus, a supercooled structure forms during cooling the wire rod to deteriorate the elongation of the wire rod. Therefore, it is preferable that an upper limit of the amount of Cr be 1.00%.

As the method for manufacturing the wire rod according to the present embodiment, both of the DLP method and the stelmor method can be employed. If the wire rod is manufactured with the stelmor method, it is more preferable that the amount of Cr be 0.50 to 1.00%. If the wire rod is manufactured with the stelmor method, the cooling rate of the wire rod is lower than that in the manufacturing with the DLP method, and thus, the elongation and the toughness of the wire rod is relatively low. In order to compensate the decreasing of the strength, it is more preferable that the lower limit of the amount of Cr be 0.50%. It is further preferable that the amount of Cr be 0.50 to 0.90%.

### (V: 0 to 0.800%)

In the wire rod according to the present embodiment, it is not necessary to include V. Therefore, a lower limit of an amount of V is 0%. However, V is an element which combines with C to precipitate as carbide in ferrite. Due to the precipitation of the carbide, the ferrite can be hardened and the wire rod can be high-strengthened. The effect can be obtained if 0.005% or more of V is included. However, if the amount of V is more than 0.800%, a coarse carbides precipitate. The coarse carbides act as the origins of cracking in working the wire rod. Therefore, it is preferable that the amount of V be 0.005 to 0.800%.

As the method for manufacturing the wire rod according to the present embodiment, both of the DLP method and the stelmor method can be employed. If the wire rod is manufactured with the stelmor method, it is more preferable that the amount of V be 0.300 to 0.500%. If the wire rod is manufactured with the stelmor method, the cooling rate of the wire rod is lower than that in the manufacturing with the DLP method, and thus, the elongation and the toughness of the wire rod is relatively low. In order to compensate the decreasing of the strength, it is more preferable that the lower limit of the amount of V be 0.300%. In addition, since micro cracks form at boundary portions of VC precipitates and base iron when a processing strain occurs, it is more preferable that an upper limit of the amount of V be 0.500%. It is further preferable that the amount of V be 0.300 to 0.400%.

### (remainder: Fe and impurity)

Remainder of the wire rod according to the present embodiment includes Fe and impurity. The impurity is a component which is incorporated by raw materials such as mineral or scrap or various factors of a manufacturing process when the steel is industrially manufactured, and is accepted within a range that does not adversely affect the property of the wire rod according to the present embodiment.

### (The average value of the grain size of a pearlite block in a cross section perpendicular to a wire rod axial direction: 23µm or less.)

In the present embodiment, a pearlite block boundary is defined as a boundary of adjacent two pearlites between which a difference in crystal orientation is 9° or higher, a pearlite block is defined as an area surrounded by the pearlite block boundary, and PBS (Pearlite Block Size) is defined as an equivalent circle diameter of the pearlite block. In the wire rod according to the present embodiment, in addition to the above-described definition of the chemical composition, an average PBS (Pearlite Block Size) in a cross section perpendicular to a wire rod axial direction is defined to 23µm or less.

If the average PBS (Pearlite Block Size) is more than 23µm, a reduction of area of the wire rod deteriorates. It is necessary that the wire rod according to the present embodiment has 30% or more of the reduction of area. In view of the past production result, it was found that 30% or more of the reduction of area was necessary to prevent breaking from causing during drawing in the drawing working of the wire rod. As a result of the inventor's consideration, it was found that there was a relationship indicated by a graph of Figure 1 between the average pearlite block size and the reduction of area. Figure 1 indicates that 30% or more of the reduction of area can be obtained when the average PBS (Pearlite Block Size) is 23µm or less. In addition, when the average PBS (Pearlite Block Size) is more than 23µm, frequency of branching of the crack end decreases. Since a branch of the crack end has an effect of suppressing crack propagation, decreasing the frequency of branching of the crack end enlarges a fracture facet to deteriorate the low-temperature elongation and the low-temperature toughness. Therefore, the average PBS (Pearlite Block Size) is 23µm or less. It is preferable that the average pearlite block size be 18µm or less.

The average value of the equivalent circle diameter of the pearlite block in any size of field of view at any position of the cross section perpendicular to the wire rod axial direction can be obtained by using EBSD device. The average PBS in the cross section perpendicular to the wire rod axial direction according to the present embodiment can be obtained by the following procedures. At first, average values (primary average values) of equivalent circle diameters of pearlite blocks in 300µm × 180µm of fields of view in each of five area consisting of
(1) a surface part (an area of which a depth from a surface of the wire rod is 30µm),
(2) a 1/4D part (an area of which a depth from the surface of the wire rod is 1/4 of a diameter D of the wire rod),
(3) a center part,
(4) a 3/4D part (an area of which a depth from the surface of the wire rod is 3/4 of a diameter D of the wire rod, i.e. an area opposite to the (2) with respect to the center part of the wire rod), and
(5) an opposite surface part (i.e. an area opposite to the (1) with respect to the center part of the wire rod),
are measured by using the EBSD device. Then, the average value (secondary average value) of the each primary average values is calculated. The secondary average value is the average PBS in the cross section perpendicular to the wire rod axial direction according to the present embodiment.

### (The number density of the pearlite block having 40µm or more of grain size in the cross section perpendicular to the wire rod axial direction is 0 to 20 pieces/mm².)

In the wire rod according to the present embodiment, in addition to the above-described definition of the chemical composition and the average value of the grain size of the pearlite block, the number density of the pearlite block having a grain size of 40µm or more in the cross section perpendicular to the wire rod axial direction is defined to 0 to 20 pieces/mm².

Since the pearlite blocks having 40µm or more of grain size act as fracture origins, the pearlite blocks having 40µm or more of grain size deteriorate the elongation and the toughness of the wire rod even if the number of the pearlite blocks having 40µm or more of grain size is small. In addition to controlling the average value of the grain size of the pearlite block, in the wire rod according to the present embodiment, it is necessary that a coarse pearlite block is prevented from forming. For these reasons, the number density of the coarse pearlite blocks is limited. Hereinafter, "pearlite block having a grain size of 40µm or more" may be referred to as "coarse pearlite block" or "coarse PB".

If the number density of the coarse pearlite blocks in the cross section perpendicular to the wire rod axial direction is more than 20 pieces/mm², the elongation and the toughness of the wire rod do not satisfy required levels. Therefore, it is necessary that the number density of the coarse pearlite blocks in the cross section perpendicular to the wire rod axial direction is limited to 0 to 20 pieces/mm². It is preferable that an upper limit of the number density of the coarse pearlite blocks in the cross section perpendicular to the wire rod axial direction be 18 pieces/mm². The less the amount of the coarse pearlite blocks are, the more preferable it is, and therefore, the lower limit of the number density of the coarse pearlite blocks in the cross section perpendicular to the wire rod axial direction is 0 pieces/mm².

The number density of the pearlite blocks having a grain size of 40µm or more in any size of field of view at any position of the cross section perpendicular to the wire rod axial direction can be obtained by using EBSD device. The number density of the pearlite blocks having 40µm or more of grain size in the cross section perpendicular to the wire rod axial direction according to the present embodiment can be obtained by the following procedures. At first, the number densities of the pearlite blocks having a grain size of 40µm or more in 300µm × 180µm of fields of view in each of five areas of
(1) a surface part (an area of which a depth from a surface of the wire rod is 30µm),
(2) a 1/4D part (an area of which a depth from the surface of the wire rod is 1/4 of a diameter D of the wire rod),
(3) a center part,
(4) a 3/4D part (an area of which a depth from the surface of the wire rod is 3/4 of a diameter D of the wire rod, i.e. an area opposite to the (2) with respect to the center part of the wire rod), and
(5) an opposite surface part (i.e. an area opposite to the (1) with respect to the center part of the wire rod),
are measured by using the EBSD device. Then, the average value of the number densities in each areas is calculated. The average value is the number density of the pearlite block having a grain size of 40µm or more in the cross section perpendicular to the wire rod axial direction according to the present embodiment.

Then, a method for manufacturing the wire rod according to the present embodiment will be described.

There are DLP method and stelmor method as the method for manufacturing the wire rod according to the present embodiment.

When the wire rod according to the present embodiment is manufactured by the stelmor method, as shown in Figure 10, (1) heating a steel piece having a chemical composition including, in terms of mass%, C: 0.70 to 0.90%; Si: 0.80 to 1.30%; Mn: 0.60 to 0.90%; P: 0.020% or less; S: 0.020% or less; N: 0.0025 to 0.0060%; Cr: 0 to 1.00%; V: 0 to 0.500%; one or more selected from the group consisting of Al: 0.005 to 0.100%, Ti: 0.003 to 0.050%, and B: 0.0005 to 0.0040%; and remainder including Fe and impurity to a rough-rolling temperature of 950 to 1040°C and then rough-rolling, (2) finish-wire-rolling at a finish-rolling temperature of 750 to 950°C, (3) coiling at a coiling temperature of 730 to 840°C, and (4) air blast cooling to a normal temperature with a cooling rate of 15°C/sec or more are performed. In this case, it is necessary that the finish-rolling temperature and a strain rate satisfy a relation of following expression 1. $\begin{matrix}13.7 \leq {log}_{10} \left\{\left(dε / dt\right) \times exp ( 63800 / \left(1.98 \times \left(T + 273.15\right)\right)\right\} \leq \\ 16.5\end{matrix}$ dε / dt expresses the strain rate during the finish-wire-rolling in terms of s⁻¹ and T expresses the finish-rolling temperature in terms of °C.

When manufacturing with stelmor method is performed, the steel piece may further include, in terms of mass%, one or more selected from the group consisting of Cr: 0.50 to 1.00%, and V: 0.300 to 0.500%.

### (The chemical composition of a steel piece used for rough-rolling: within defined range as described above.)

When the wire rod according to the present embodiment is manufactured by the stelmor method, it is necessary that the chemical composition of a steel piece used for rough-rolling is within defined range as described above. The defined range is narrower than the above-described defined range of the chemical composition of the wire rod according to the present embodiment. The stelmor method is a manufacturing method in which air blast cooling is performed after coiling, and the cooling rate by the air blast cooling is lower than a cooling rate of a direct heat treatment by a molten salt in a DLP method described below. When the cooling rate is low, the elongation and the toughness of the wire rod finally obtained are relatively low. Therefore, in a case in which the wire rod according to the present embodiment is manufactured by the stelmor method, it is necessary that the amount of C, Mn, and Si which are alloy elements for enhancing the elongation and the toughness are more than that in a case of performing the direct heat treatment by the molten salt in the DLP method. In addition, in a case in which Ca and V are included in order to enhance the property of the wire rod when the wire rod according to the present embodiment is manufactured with stelmor method, it is preferable that the amount of Cr and V be also more than that in the case of performing the direct heat treatment by the molten salt in the DLP method.

### (heating temperature of the steel piece before rough-rolling)

In the method for manufacturing the wire rod according to the present embodiment with stelmor method, a heating temperature of the steel piece before the rough-rolling (rough-rolling temperature) is 950 to 1040°C. If the heating temperature of the steel piece before rough-rolling is lower than 950°C, roll reaction forth in wire rod rolling may rapidly increase to cause trouble of the equipment such as cracking of roll. Therefore, the heating temperature of the steel piece before the rough-rolling is 950°C or more. On the other hand, if the heating temperature of the steel piece before the rough-rolling is more than 1040°C, solutionizing of aluminum nitride (AlN) precipitated in the steel piece progresses excessively. As described above, AlN act as the nucleuses of precipitation of the austenite to contribute to refine the grain size of the austenite. The grain size of the pearlite of the wire rod finally obtained can be refined by refining the grain size of the austenite of the wire rod during manufacturing stage. However, if the solutionizing of AlN progresses excessively, coarsening the grain size of the austenite progresses. In this case, PBS of the wire rod is coarsened after manufacturing the wire rod. In this case, the average value of the grain size of the pearlite block in the cross section perpendicular to the wire rod axial direction becomes more than 23µm, and/or the number density of the pearlite block having 40µm or more of the grain size becomes more than 20 pieces/mm². In order to avoid such phenomenon from causing, the heating temperature of the steel piece before the rough-rolling is 1040°C or lower.

### (a temperature in finish-wire-rolling: 750 to 950°C)

In the method for manufacturing the wire rod according to the present embodiment with stelmor method, finish-wire-rolling is performed at a temperature range of 750 to 950°C. If the temperature in the finish-wire-rolling (finish-rolling temperature) is less than 750°C, roll reaction forth during rolling may increase to cause trouble of the equipment such as cracking of roll, and thus, the temperature in the finish-wire-rolling is 750°C or more. On the other hand, if the temperature during the finish-wire-rolling is more than 900°C, the grain size of the austenite coarsens. In this case, the average value of the grain size of the pearlite block in the cross section perpendicular to the wire rod axial direction becomes more than 23µm, and/or the number density of the pearlite blocks having 40µm or more of the grain size becomes more than 20 pieces/mm². The elongation of the wire rod is deteriorated by coarsening the pearlite block. In order to avoid such phenomenon, the temperature during the finish-wire-rolling is 900°C or lower.

### (relation between the finish-rolling temperature and a strain rate in the finish-wire-rolling: 13.7 ≤ log₁₀ Z ≤ 16.5)

In addition, in the method for manufacturing the wire rod according to the present embodiment with stelmor method, it is necessary that a relation between the finish-rolling temperature and a strain rate in the finish-wire-rolling is defined. Specifically, it is necessary that common logarithm (log₁₀ Z) of Z value (Zener-Hollomon parameter) is 13.7 to 16.5, in which the Z value is obtained by substituting a strain rate of the wire rod at the finish-wire-rolling dε / dt, an activation energy of plastic deformation of the wire rod Q, and the finish-rolling temperature at the finish-wire-rolling T into the following expression 2 which indicates Zener-Hollomon expression. $Z = \left(dε / dt\right) \times exp \left(Q / RT\right)$ "dε / dt" expresses the strain rate in terms of s⁻¹. "R" is gas constant and the value thereof is 1.98 cal/mol·deg. "T" expresses the finish-rolling temperature in terms of K. If the term of the finish-rolling temperature is °C, it is necessary that "T" in the expression 2 is replaced by "(T + 273.15)". "Q" expresses the activation energy of the plastic deformation of the wire rod. It is assumed that the activation energy of the plastic deformation of the wire rod according to the present embodiment having the above-described chemical composition is 63800 cal/mol.

In the method for manufacturing according to the present embodiment, the strain rate of the wire rod at the finish-wire-rolling dε / dt can be obtained by the following expression. $dε / dt = ε \times 2 \times π \times \left(N / 60\right) \times {L}_{d}$ $ε = ln \left(h 2 / h 1\right)$ ${L}_{d} = {\left(r / Δh\right)}^{1 / 2}$ $Δh = h 1 - h 2$ "ε" is an amount of strain during the finish-wire-rolling and is a dimensionless parameter. "h1" is a diameter of the wire rod before the finish-wire-rolling in terms of mm, and "h2" is a diameter of the wire rod after the finish-wire-rolling in terms of mm. "N" is a number of revolution of a roll performing the finish-wire-rolling in terms of rpm. "L_{d}" is a projected roll contact length during the finish-wire-rolling in terms of mm. The projected roll contact length is the length of an area, at which the roll contacts with a rolled material (wire rod) during the rolling, along the rolling direction. "r" is a radius of the roll at the finish-wire-rolling in terms of mm. "Δh" is a rolling reduction during the finish-wire-rolling in terms of mm. As shown in expressions 3 to 6, the strain rate is a rolling condition depending on both of rolling speed and rolling reduction.

As a result of the inventor's consideration, it was found that there was a relationship indicated in Figure 2 between the Z value at the finish-wire-rolling and the average pearlite block size of the wire rod finally obtained. As shown in Figure 2, in order to control the average pearlite block size in the cross section perpendicular to the wire rod axial direction to 23µm or less, it is necessary that log₁₀ Z be 13.7 or more. In addition, in order to control the number density of the coarse pearlite blocks having 40µm or more of grain size to 0 to 20 pieces/mm², as is the case with that, it is necessary that log₁₀ Z is 13.7 or more. On the other hand, in view of the equipment capacity, it is difficult to set log₁₀ Z to more than 16.5. As shown in the Zener-Hollomon expression, in order to increase Z value, it is necessary to decrease the rolling temperature and increase the strain rate. Therefore, in the method for manufacturing the wire rod according to the present embodiment with stelmor method, the upper limit of log₁₀ Z is 16.5. It is preferable that log₁₀ Z be 14.0 to 16.0. If log ₁₀ Z is lower than above-described range, the average value of the grain size of the pearlite block in the cross section perpendicular to the wire rod axial direction becomes more than 23µm, and/or the number density of the pearlite block having 40µm or more of the grain size becomes more than 20 pieces/mm².

The speed of the finish-wire-rolling (finish rolling speed) is not limited as long as log₁₀ Z is within the range of 13.7 to 16.5. It is preferable that, if a wire rod having a diameter of 12mm or more is manufactured, the speed of the finish-wire-rolling be 15.5 to 25.2 m/sec. If the speed of the finish-wire-rolling is less than 15.5 m/sec, the strain rate decreases. In this case, PBS may not be sufficiently reduced. Therefore, it is preferable that the speed of the finish-wire-rolling be 15.5 m/sec or more. On the other hand, if the speed of the finish-wire-rolling is more than 25.2 m/sec, exotherm during working may increase to coarsen the grain size of austenite. Also in this case, PBS cannot be refined. As shown in above-described expressions 3 to 6, when a wire rod of which the diameter is not 12 mm, it is necessary that the speed of the finish-wire-rolling is arbitrarily changed from the above-described range so that log₁₀ Z is within the range of 13.7 to 16.5.

### (coiling temperature: 730 to 840°C)

### (air blast cooling rate after coiling: 15°C/sec or more)

In the method for manufacturing the wire rod according to the present embodiment with stelmor method, after the finish-wire-rolling, the wire rod is coiled at a temperature of 730 to 840°C, and then, air blast cooling is performed with a cooling rate of 15°C/sec or more. If the coiling temperature is lower than 730°C, the amount of scale decreases to deteriorate mechanical descalability, and thus, the coiling temperature is 730°C or more. If the coiling temperature is higher than 840°C, the grain size of the austenite increases. In this case, the grain size of the pearlite block of the wire rod finally obtained cannot be controlled to 23µm or less, and/or the number density of the pearlite blocks having 40µm or more of the grain size becomes more than 20 pieces/mm². Therefore, the coiling temperature is 840°C or lower. It is preferable that the coiling temperature be 750 to 820°C.

The wire rod after the coiling is cooled by air blast cooling to a normal temperature. The normal temperature basically indicates a temperature range of 5 to 35°C as defined in JIS Z 8703. In the case, if the cooling rate is lower than 15°C/sec (i.e. slow cooling), the grain size of austenite increases, and thus, the average value of the grain size of the pearlite block in the cross section perpendicular to the wire rod axial direction becomes more than 23µm, and/or the number density of the pearlite block having 40µm or more of the grain size becomes more than 20 pieces/mm². As a result, the elongation of the wire rod finally obtained deteriorates. Therefore, the cooling rate at the air blast cooling is 15°C/sec or more. It is preferable that the cooling rate at the air blast cooling be 25°C/sec or more. Although it is not necessary to define the upper limit of the cooling rate at the air blast cooling, in view of the equipment capacity, the upper limit is about 50°C/sec.

When the wire rod according to the present embodiment is manufactured by the DLP method, (1) heating a steel piece having a chemical composition including, in terms of mass%, C: 0.60 to 1.20%; Si: 0.30 to 1.30%; Mn: 0.30 to 0.90%; P: 0.020% or less; S: 0.020% or less; N: 0.0025 to 0.0060%; Cr: 0 to 1.00%; V: 0 to 0.500%; one or more selected from the group consisting of Al: 0.005 to 0.100%, Ti: 0.003 to 0.050%, and B: 0.0005 to 0.0040%; and remainder including Fe and impurity to a temperature of 950 to 1040°C and wire rod rolling, (2) coiling at a temperature range of 750 to 800°C, and (3) direct heat treating with 500 to 600°C of a molten salt just after termination of the coiling are performed.

When the wire rod according to the present embodiment is manufactured with DLP method, the steel piece, which is raw material, may further include, in terms of mass%, one or more selected from the group consisting of Cr: 0.10 to 1.00%, and V: 0.005 to 0.800%.

### (a chemical composition of a steel piece used for wire rod rolling: within defined range as described above)

When the wire rod according to the present embodiment is manufactured by the DLP method, it is necessary that a chemical composition of a steel piece used for wire rod rolling is within defined range as described above. The defined range is equal to the above-described defined range of the chemical composition of the wire rod according to the present embodiment. A method for manufacturing with DLP method has an advantage that a wire rod having excellent elongation and toughness can be obtained from a steel piece of which alloy elements for enhancing the elongation and the toughness is relatively low. However, direct heat treatment with molten salt is essential the for the method for manufacturing with the DLP method, and thus, in order to bring the method for manufacturing with the DLP method into operation, much more equipment is required than that with the stelmor method.

### (heating temperature in wire rod rolling: 950 to 1040°C)

When the wire rod according to the present embodiment is manufactured by the DLP method, the heating temperature of the wire rod before wire rod rolling the steel piece is 950 to 1040°C. If the heating temperature is lower than 950°C, roll reaction forth during the wire rod rolling may considerably increase to cause troubles in equipments such as cracking of roll, and thus, the heating temperature before the wire rod rolling is 950°C or more. On the other hand, if the heating temperature before the wire rod rolling is higher than 1040°C, solutionizing of aluminum nitride (AlN) precipitated in the steel piece progresses, and thus, coarsening the grain size of the austenite progresses to coarsen the pearlite block size (PBS) of the wire rod finally obtained. In this case, the average value of the grain size of the pearlite block in the cross section perpendicular to the wire rod axial direction becomes more than 23µm, and/or the number density of the pearlite blocks having 40µm or more of the grain size becomes more than 20 pieces/mm². In order to avoid such phenomenon from causing, the heating temperature before the wire rod rolling is 1040°C or lower. It is preferable that the heating temperature before the wire rod rolling be 980 to 1030°C. The finish temperature at the wire rod rolling is not limited, and thus, a reasonable temperature can be arbitrarily selected.

### (coiling temperature: 750 to 850°C)

When the wire rod according to the present embodiment is manufactured by the DLP method, coiling temperature after the wire rod rolling is 750 to 850°C. If the coiling temperature is lower than 750°C, unevenness along longitudinal direction of the wire rod regarding tensile strength increases after isothermal transformation in the following isothermal transformation treating. Therefore, the coiling temperature is 750°C or higher. If the coiling temperature is higher than 800°C, the grain size of austenite increases. In this case, the grain size of the pearlite block of the wire rod finally obtained cannot be controlled to 23µm or less and the number density of the pearlite block having 40µm or more of the grain size cannot be controlled to be 20 pieces/mm² or less, and thus, the coiling temperature is 800°C or lower.

### (method for isothermal transformation treating: direct heat treating)

### (isothermal transformation treating temperature: 500 to 600°C)

When the wire rod according to the present embodiment is manufactured by the DLP method, immediately after coiling the wire rod, the wire rod is immersed into 500 to 600°C of molten salt to perform isothermal transformation treating. If the isothermal transformation treating temperature is lower than 500°C, many amount of non-pearlite structure forms at the surface part of the wire rod. In this case, unevenness of processing strain occurs at boundary between pearlite structure forming at internal part of the wire rod and the non-pearlite structure at the surface part, and the unevenness may cause breaking during wire drawing stage. Therefore, the isothermal transformation treating temperature is 500°C or higher. If the isothermal transformation treating temperature is higher than 600°C, operational problems such as increasing heat deformation of the equipment occurs, and thus, the isothermal transformation treating temperature is 600°C or lower. In addition, it is necessary that the isothermal transformation treatment is performed with direct heat treatment (online heat treatment). If the direct heat treatment is not performed (i.e. the isothermal transformation treatment is performed with offline heat treatment), reheating included in the offline heat treatment causes growth of y grain. The phenomenon prevents the grain size of PBS of the wire rod from being controlled to 23µm or less.

### [Examples]

Hereinafter, examples of the present invention will be described. The conditions in manufacturing the examples are an example condition employed to confirm the operability and the effects of the present invention, so the present invention is not limited to the example condition. The present invention can employ various types of conditions as long as the conditions do not depart from the scope of the present invention and can achieve the object of the present invention.

### (Example)

Hereinafter, examples by a method for manufacturing with stelmor method will be described.

At first, molten steel having chemical composition shown in Table 1-1 was continuously casted so as to be a cast bloom of 300mm × 500mm, and the cast bloom is rolled so as to be a steel billet of 122mm square by blooming. Then, the steel billet was heated to a heating temperature shown in Table 1-2 and rolled under a condition shown in the Table 1-2 to obtain a wire rod of 12mmϕ. A radius of a roll in finish-wire-rolling was 75.5mm. No. S1 to S16 are examples which satisfy the condition according to the present invention and No. S17 to S41 are comparative examples which do not satisfy the condition according to the present invention.

A tensile test pieces shown in Figure 3 were manufactured from the rolled wire rods. Tensile test was performed to the tensile test pieces at a low temperature atmosphere of -40°C while controlling the temperature using dry ice and alcohol to measure tensile strength and elongation at -40°C of the wire rod.

In addition, a charpy impact test pieces defined in JIS Z 2202 were extracted from the above-described wire rods in a manner of extracting shown in Figure 4 to manufacture 5mm subsize 2mm U-notch charpy impact test pieces. Charpy impact test at -40°C was performed to the charpy impact test pieces to obtain impact value of the wire rods at a temperature of -40°C, which was similar to actual using environment temperature of PC dike of PC-type LNG tank.

The average PBS (Pearlite Block Size) of the wire rod was obtained by the following procedures. At first, average values (primary average values) of an equivalent circle diameter of a pearlite block in 300µm × 180µm of fields of view in each of five area of
(1) a surface part (an area of which a depth from a surface of the wire rod was 30µm),
(2) a 1/4D part (an area of which a depth from the surface of the wire rod was 1/4 of a diameter D of the wire rod),
(3) a center part,
(4) a 3/4D part (an area of which a depth from the surface of the wire rod was 3/4 of a diameter D of the wire rod, i.e. an area opposite to the (2) with respect to the center part of the wire rod), and
(5) an opposite surface part (i.e. an area opposite to the (1) with respect to the center part of the wire rod),
were measured by using the EBSD device. Then, the average value (secondary average value) of the each primary average values was calculated. The secondary average value was assumed as the average PBS in the cross section perpendicular to the wire rod axial direction. During measuring with EBSD device, a boundary of adjacent two pearlites between which a difference in crystal orientation was 9° or higher was judged as a pearlite block boundary.

The number density of the coarse pearlite blocks of the wire rod was obtained by the following procedures. At first, number densities of the pearlite block having 40µm or more of grain size in 300µm × 180µm of fields of view in each of five area of
(1) a surface part (an area of which a depth from a surface of the wire rod was 30µm),
(2) a 1/4D part (an area of which a depth from the surface of the wire rod was 1/4 of a diameter D of the wire rod),
(3) a center part,
(4) a 3/4D part (an area of which a depth from the surface of the wire rod was 3/4 of a diameter D of the wire rod, i.e. an area opposite to the (2) with respect to the center part of the wire rod), and
(5) an opposite surface part (i.e. an area opposite to the (1) with respect to the center part of the wire rod),
were measured by using the EBSD device. Then, the average value of the each number densities was calculated. The average value was assumed as the number density of the pearlite blocks having 40µm or more of grain size in the cross section perpendicular to the wire rod axial direction.

**[Table 1-1]**

| No | CHEMICAL COMPOSITION UNIT: mass% | | | | | | | | | | |
|---|---|---|---|---|---|---|---|---|---|---|---|
| | C | Si | Mn | P | S | Al | Ti | B | N | Cr | V |
| S1 | 0.70 | 0.80 | 0.76 | 0.017 | 0.010 | 0.020 | 0.038 | 0.0024 | 0.0031 | 0.50 | - |
| S2 | 0.82 | 0.85 | 0.72 | 0.015 | 0.010 | 0.060 | 0.040 | 0.0037 | 0.0036 | 1.00 | - |
| S3 | 0.88 | 0.90 | 0.72 | 0.008 | 0.006 | - | 0.048 | - | 0.0047 | - | - |
| S4 | 0.88 | 1.00 | 0.73 | 0.006 | 0.009 | 0.025 | 0.005 | 0.0035 | 0.0041 | 0.50 | 0.320 |
| S5 | 0.90 | 0.90 | 0.80 | 0.009 | 0.007 | 0.042 | 0.010 | 0.0019 | 0.0060 | 0.50 | 0.310 |
| S6 | 0.85 | 0.85 | 0.90 | 0.010 | 0.010 | 0.032 | - | 0.0020 | 0.0045 | - | 0.400 |
| S7 | 0.90 | 0.85 | 0.72 | 0.012 | 0.000 | 0.033 | 0.025 | 0.0040 | 0.0035 | 0.60 | - |
| S8 | 0.87 | 1.30 | 0.70 | 0.015 | 0.005 | 0.040 | 0.035 | 0.0036 | 0.0025 | - | - |
| S9 | 0.87 | 0.95 | 0.71 | 0.015 | 0.006 | 0.060 | - | 0.0028 | 0.0036 | - | - |
| S10 | 0.87 | 0.96 | 0.74 | 0.011 | 0.009 | 0.060 | - | - | 0.0025 | - | 0.500 |
| S11 | 0.87 | 0.98 | 0.75 | 0.020 | 0.007 | - | 0.015 | 0.0030 | 0.0042 | 0.66 | - |
| S12 | 0.90 | 1.30 | 0.60 | 0.016 | 0.009 | 0.005 | 0.011 | 0.0029 | 0.0036 | 0.56 | - |
| S13 | 0.90 | 0.82 | 0.70 | 0.009 | 0.008 | 0.035 | 0.005 | - | 0.0039 | - | - |
| S14 | 0.90 | 0.82 | 0.70 | 0.009 | 0.008 | - | - | 0.0035 | - | - | - |
| S15 | 0.90 | 0.85 | 0.74 | 0.007 | 0.010 | 0.028 | 0.023 | 0.0033 | 0.0029 | 0.80 | 0.400 |
| S16 | 0.90 | 0.85 | 0.74 | 0.007 | 0.010 | 0.028 | 0.023 | 0.0033 | 0.0029 | 0.80 | 0.400 |
| S17 | 0.70 | 0.85 | 0.35 | 0.020 | 0.022 | 0.005 | - | - | - | - | - |
| S18 | 0.82 | 0.75 | 0.81 | 0.022 | 0.019 | 0.030 | - | - | - | - | - |
| S19 | 0.50 | 0.80 | 0.76 | 0.017 | 0.010 | 0.020 | 0.038 | 0.0024 | 0.0031 | 0.50 | - |
| S20 | 1.03 | 0.85 | 0.74 | 0.007 | 0.010 | 0.028 | 0.023 | 0.0033 | 0.0029 | 0.80 | 0.400 |
| S21 | 0.92 | 0.91 | 0.75 | 0.035 | 0.023 | 0.033 | - | - | - | - | - |
| S22 | 0.82 | 1.38 | 0.72 | 0.015 | 0.010 | 0.060 | 0.040 | 0.0037 | 0.0036 | 1.00 | - |
| S23 | 0.82 | 0.85 | 1.10 | 0.015 | 0.010 | 0.060 | 0.040 | 0.0037 | 0.0036 | 1.00 | - |
| S24 | 0.82 | 0.85 | 0.30 | 0.015 | 0.010 | 0.060 | 0.040 | 0.0037 | 0.0036 | 1.00 | - |
| S25 | 0.82 | 0.85 | 0.72 | 0.042 | 0.010 | 0.060 | 0.040 | 0.0037 | 0.0036 | 1.00 | - |
| S26 | 0.82 | 0.85 | 0.72 | 0.015 | 0.038 | 0.060 | 0.040 | 0.0037 | 0.0036 | 1.00 | - |
| S27 | 0.82 | 0.85 | 0.72 | 0.015 | 0.010 | 0.120 | 0.040 | 0.0037 | 0.0036 | 1.00 | - |
| S28 | 0.82 | 0.85 | 0.72 | 0.015 | 0.010 | 0.060 | 0.120 | 0.0037 | 0.0036 | 1.00 | - |
| S29 | 0.82 | 0.85 | 0.72 | 0.015 | 0.010 | 0.060 | 0.040 | 0.0055 | 0.0036 | 1.00 | - |
| S30 | 0.82 | 0.85 | 0.72 | 0.015 | 0.010 | 0.001 | 0.040 | 0.0037 | 0.0036 | 1.00 | - |
| S31 | 0.82 | 0.85 | 0.72 | 0.015 | 0.010 | 0.060 | 0.001 | 0.0037 | 0.0036 | 1.00 | - |
| S32 | 0.82 | 0.85 | 0.72 | 0.015 | 0.010 | 0.060 | 0.040 | 0.0002 | 0.0036 | 1.00 | - |
| S33 | 0.82 | 0.85 | 0.72 | 0.015 | 0.010 | 0.060 | 0.040 | 0.0037 | 0.0036 | 1.50 | - |
| S34 | 0.82 | 0.85 | 0.72 | 0.015 | 0.010 | 0.060 | 0.040 | 0.0037 | 0.0036 | 1.00 | 0.620 |
| S35 | 0.82 | 0.85 | 0.72 | 0.015 | 0.010 | 0.060 | 0.040 | 0.0037 | 0.0036 | 1.00 | - |
| S36 | 0.82 | 0.85 | 0.72 | 0.015 | 0.010 | 0.060 | 0.040 | 0.0037 | 0.0036 | 1.00 | - |
| S37 | 0.82 | 0.85 | 0.72 | 0.015 | 0.010 | 0.060 | 0.040 | 0.0037 | 0.0036 | 1.00 | - |
| S38 | 0.82 | 0.85 | 0.72 | 0.015 | 0.010 | 0.060 | 0.040 | 0.0037 | 0.0036 | 1.00 | - |
| S39 | 0.82 | 0.85 | 0.72 | 0.015 | 0.010 | 0.060 | 0.040 | 0.0037 | 0.0036 | 1.00 | - |
| S40 | 0.82 | 0.85 | 0.72 | 0.015 | 0.010 | 0.060 | 0.040 | 0.0037 | 0.0036 | 1.00 | - |
| S41 | 0.82 | 0.85 | 0.72 | 0.015 | 0.010 | 0.060 | 0.040 | 0.0037 | 0.0036 | 1.00 | - |

### UNDERLINED VALUE IS OUT OF RANGE OF PRESENT INVENTION

**[Table 1-2]**

| No | HEATING TEMPERATURE BEFORE ROUGH-ROLLING | FINISH-ROLLING TEMPERATURE | STRAIN RATE IN THE FINISH-WIRE-ROLLING | log₁₀Z | COILING TEMPERATURE | COOLING RATE | REMARKS |
|---|---|---|---|---|---|---|---|
| | °C | °C | s⁻¹ | | °C | °C/s | |
| S1 | 950 | 750 | 607 | 16.5 | 730 | 15 | |
| S2 | 950 | 800 | 607 | 15.8 | 750 | 15 | |
| S3 | 960 | 750 | 607 | 16.5 | 730 | 22 | |
| S4 | 970 | 800 | 607 | 15.8 | 780 | 20 | |
| S5 | 980 | 800 | 607 | 15.8 | 790 | 15 | |
| S6 | 980 | 850 | 607 | 15.2 | 800 | 16 | |
| S7 | 1000 | 900 | 607 | 14.7 | 790 | 17 | |
| S8 | 1000 | 850 | 607 | 15.2 | 785 | 15 | |
| S9 | 1000 | 850 | 607 | 15.2 | 800 | 15 | EXAMPLE |
| S10 | 1020 | 850 | 607 | 15.2 | 790 | 20 | |
| S11 | 1030 | 800 | 607 | 15.8 | 790 | 20 | |
| S12 | 1030 | 800 | 607 | 15.8 | 795 | 22 | |
| S13 | 1040 | 750 | 607 | 16.5 | 730 | 20 | |
| S14 | 1040 | 750 | 607 | 16.5 | 730 | 20 | |
| S15 | 1040 | 900 | 607 | 14.7 | 830 | 25 | |
| S16 | 1040 | 900 | 607 | 14.7 | 830 | 25 | |
| S17 | 1080 | 1050 | 371 | 13.2 | 880 | 5 | |
| S18 | 1080 | 1000 | 371 | 13.6 | 850 | 10 | |
| S19 | 950 | 750 | 371 | 16.3 | 730 | 15 | |
| S20 | 1040 | 900 | 371 | 14.5 | 800 | 25 | |
| S21 | 1100 | 1100 | 371 | 12.8 | 900 | 12 | |
| S22 | 950 | 800 | 607 | 15.8 | 750 | 15 | |
| S23 | 950 | 800 | 607 | 15.8 | 750 | 15 | |
| S24 | 950 | 800 | 607 | 15.8 | 750 | 15 | |
| S25 | 950 | 800 | 607 | 15.8 | 750 | 15 | |
| S26 | 950 | 800 | 607 | 15.8 | 750 | 15 | |
| S27 | 950 | 800 | 607 | 15.8 | 750 | 15 | |
| S28 | 950 | 800 | 607 | 15.8 | 750 | 15 | |
| S29 | 950 | 800 | 607 | 15.8 | 750 | 15 | |
| S30 | 950 | 800 | 607 | 15.8 | 750 | 15 | |
| S31 | 950 | 800 | 607 | 15.8 | 750 | 15 | COMPARATIVE EXAMPLE |
| S32 | 950 | 800 | 607 | 15.8 | 750 | 15 | |
| S33 | 950 | 800 | 607 | 15.8 | 750 | 15 | |
| S34 | 950 | 800 | 607 | 15.8 | 750 | 15 | |
| S35 | 1150 | 800 | 607 | 15.8 | 750 | 15 | |
| S36 | 950 | 720 | 607 | 16.9 | 750 | 15 | |
| S37 | 950 | 1150 | 607 | 12.6 | 750 | 15 | |
| S38 | 950 | 800 | 607 | 15.8 | 890 | 15 | |
| S39 | 950 | 800 | 607 | 15.8 | 750 | 7 | |
| S40 | 950 | 950 | 607 | 14.2 | 750 | 15 | |
| S41 | 950 | 900 | 42 | 13.5 | 750 | 15 | |

| | | | | | | | |
|---|---|---|---|---|---|---|---|
| UNDERLINED VALUE IS OUT OF RANGE OF PRESENT INVENTION FINAL DIAMETER: 12mm ACTIVATION ENERGY OF PLASTIC DEFORMATION: 63800cal/mol | | | | | | | |

The heating temperature, the finishing temperature, and the coiling temperature of the examples were within the adequate temperature range. Therefore, the pearlite block of the example was refined and the average PBS and the number density of the coarse PB of the example were controlled in the adequate level. On the other hand, the average PBS and the number density of the coarse PB of the comparative examples of which the heating temperature, the finishing temperature, and/or the coiling temperature were higher than the adequate temperature range were out of range defined by the present invention. The examples demonstrated better property than the comparative examples in low-temperature strength, low-temperature toughness, and room-temperature toughness. In example S36, the finish-rolling temperature was lower than the adequate temperature range, and thus, mill load increased to prevent rolling from performing.

Figure 5A shows SEM picture of the pearlite block of the example and Figure 5B shows SEM picture of the pearlite block of the comparative example. It could be found from the SEM pictures that the grain size of the pearlite block of the example was smaller than the grain size of the pearlite block of the comparative example.

Figure 6 shows a result of tensile test at -40°C of the example (No. S6) and the comparative example (No. S17). It could be found that the elongation of the example was higher and better than the elongation of the comparative example in low-temperature atmosphere of -40°C. In addition, it could be found from Table 2 that the elongation of the example tended to be higher than the elongation of the comparative example. It was assumed that the difference in elongation was caused by the difference in the grain size of the pearlite block shown in Figure 5A and Figure 5B.

Next, examples by a method for manufacturing with DLP method will be described hereinafter.

At first, molten steel having chemical composition shown in Table 3 was continuously casted so as to be a cast bloom of 300mm × 500mm, and the cast bloom was rolled so as to be a steel billet of 122mm square. Then, the steel billet was heated to a heating temperature shown in Table 3 and rolled, coiled and heat treated using molten salt under a condition shown in the Table 3 to obtain a wire rod of 12mmϕ. No. D1 to D16 and No. D30 to D36 were manufactured with a heat treatment (direct heat treatment) in which they were immersed into the molten salt without reheating after coiling. No. D17 to D29 were coiled under conditions shown in the Table 3, and then, subjected to a heat treatment (offline heat treatment) in which they were reheated to 950°C and subjected to lead patenting treatment.

Tensile strength at -40°C, elongation at -40°C, and impact value at -40°C of the above-described wire rods were obtained. The test methods for obtaining the values were same to each test methods performed to the above-described No. S1 to No. S41. In addition, charpy impact test at room temperature was performed to the above-described wire rods to obtain impact value of the wire rods at the room temperature. The method for performing the charpy impact test at the room temperature was same to the above-described method for performing the charpy impact test at -40°C except test temperature. The average PBS and the number density of the coarse pearlite blocks of the above-described wire rod were measured.

**[Table 3-1]**

| No | CHEMICAL COMPOSITION UNIT: mass% | | | | | | | | | | | HEATING TEMPERATURE BEFORE WIRE ROD ROLLING | COILING TEMPERATURE | ONLINE HEAT TREATMENT TEMPERATURE | REMARKS |
|---|---|---|---|---|---|---|---|---|---|---|---|---|---|---|---|
| | C | Si | Mn | P | S | Al | Ti | B | N | Cr | V | °C | °C | °C | |
| D1 | 0.60 | 0.80 | 0.76 | 0.017 | 0.010 | 0.020 | 0.038 | 0.0024 | 0.0031 | - | - | 950 | 750 | 500 | EXAMPLE |
| D2 | 0.82 | 0.85 | 0.72 | 0.015 | 0.010 | 0.060 | 0.040 | 0.0037 | 0.0036 | - | 0.120 | 950 | 750 | 500 | |
| D3 | 0.88 | 0.90 | 0.72 | 0.008 | 0.006 | 0.030 | 0.048 | 0.0039 | 0.0047 | - | - | 960 | 780 | 520 | |
| D4 | 0.88 | 1.00 | 0.73 | 0.006 | 0.009 | 0.025 | 0.005 | 0.0035 | 0.0041 | 0.27 | 0.320 | 970 | 780 | 520 | |
| D5 | 0.90 | 0.90 | 0.80 | 0.009 | 0.007 | 0.042 | 0.010 | - | 0.0060 | 0.23 | 0.210 | 980 | 790 | 520 | |
| D6 | 0.92 | 0.85 | 0.90 | 0.010 | 0.010 | 0.032 | 0.018 | 0.0020 | 0.0045 | - | 0.030 | 980 | 800 | 520 | |
| D7 | 0.92 | 0.85 | 0.72 | 0.012 | 0.000 | 0.033 | - | 0.0040 | 0.0025 | 0.15 | - | 1000 | 790 | 550 | |
| D8 | 0.95 | 1.30 | 0.70 | 0.015 | 0.005 | - | 0.035 | 0.0036 | 0.0035 | - | - | 1000 | 785 | 550 | |
| D9 | 0.95 | 0.95 | 0.71 | 0.015 | 0.006 | 0.085 | 0.031 | 0.0028 | 0.0036 | - | - | 1000 | 800 | 550 | |
| D10 | 0.98 | 0.96 | 0.74 | 0.011 | 0.009 | 0.060 | - | - | 0.0025 | - | 0.120 | 1020 | 790 | 550 | |
| D11 | 0.98 | 0.98 | 0.75 | 0.013 | 0.007 | 0.032 | - | 0.0030 | 0.0042 | 0.16 | - | 1030 | 790 | 560 | |
| D12 | 0.98 | 1.00 | 0.40 | 0.016 | 0.009 | 0.005 | 0.011 | 0.0029 | 0.0036 | 0.41 | - | 1030 | 795 | 560 | |
| D13 | 1.00 | 0.82 | 0.38 | 0.009 | 0.008 | 0.035 | 0.005 | - | 0.0039 | - | - | 1040 | 800 | 575 | |
| D14 | 1.18 | 0.85 | 0.35 | 0.020 | 0.010 | 0.028 | 0.023 | 0.0033 | 0.0029 | 0.48 | 0.010 | 1040 | 800 | 575 | |
| D15 | 0.98 | 0.98 | 0.75 | 0.013 | 0.007 | 0.032 | 0.040 | 0.0030 | 0.0042 | 0.16 | - | 1030 | 790 | 560 | |
| D16 | 1.00 | 0.85 | 0.35 | 0.020 | 0.010 | - | - | 0.0038 | 0.0029 | 0.48 | 0.010 | 1040 | 800 | 575 | |

**[Table 3-2]**

| No | CHEMICAL COMPOSITION UNIT: mass% | | | | | | | | | | | HEATING TEMPERATURE BEFORE WIRE ROD ROLLING | COILING TEMPERATURE | ONLINE HEAT TREATMENT TEMPERATURE | REMARKS |
|---|---|---|---|---|---|---|---|---|---|---|---|---|---|---|---|
| | C | Si | Mn | P | S | Al | Ti | B | N | Cr | V | °C | °C | °C | |
| D17 | 0.64 | 0.80 | 0.76 | 0.017 | 0.010 | 0.020 | 0.038 | 0.0024 | 0.0031 | - | - | 950 | 750 | 500 | COMPARATIVE EXAMPLE |
| D18 | 0.82 | 0.32 | 0.72 | 0.015 | 0.010 | 0.060 | 0.040 | 0.0037 | 0.0036 | - | 0.120 | 950 | 750 | 500 | |
| D19 | 0.88 | 0.63 | 0.72 | 0.008 | 0.006 | 0.030 | 0.048 | 0.0039 | 0.0047 | - | - | 960 | 780 | 520 | |
| D20 | 0.83 | 0.85 | 0.35 | 0.020 | 0.022 | 0.024 | 0.110 | - | 0.0045 | 0.22 | - | 1080 | 850 | 560 | |
| D21 | 0.87 | 0.75 | 0.81 | 0.022 | 0.019 | 0.030 | 0.160 | - | 0.0040 | - | 0.520 | 1080 | 850 | 565 | |
| D22 | 0.88 | 0.91 | 0.75 | 0.035 | 0.023 | - | - | - | - | - | - | 1100 | 850 | 550 | |
| D23 | 0.91 | 0.92 | 0.73 | 0.018 | 0.032 | 0.041 | 0.060 | 0.0030 | 0.0035 | 0.32 | - | 1100 | 850 | 550 | |
| D24 | 0.92 | 0.85 | 0.25 | 0.023 | 0.026 | 0.120 | 0.210 | 0.0025 | 0.0045 | 0.61 | - | 1120 | 850 | 563 | |
| D25 | 0.95 | 0.88 | 0.60 | 0.032 | 0.011 | 0.027 | 0.340 | - | 0.0051 | 0.41 | - | 1120 | 860 | 570 | |
| D26 | 0.98 | 1.31 | 0.45 | 0.025 | 0.015 | 0.023 | 0.110 | - | 0.0023 | 0.32 | 0.100 | 1130 | 860 | 570 | |
| D27 | 0.95 | 1.30 | 0.70 | 0.015 | 0.005 | - | 0.035 | 0.0036 | 0.0015 | - | - | 1130 | 850 | 570 | |
| D28 | 1.05 | 1.20 | 0.85 | 0.027 | 0.019 | 0.027 | 0.190 | 0.0054 | 0.0037 | - | 0.250 | 1130 | 860 | 575 | |
| D29 | 1.10 | 0.96 | 0.79 | 0.019 | 0.011 | 0.025 | 0.230 | - | 0.0073 | - | 0.330 | 1135 | 860 | 580 | |

| No | CHEMICAL COMPOSITION UNIT: mass% | | | | | | | | | | | HEATING TEMPERATURE BEFORE WIRE ROD ROLLING | COILING TEMPERATURE | ONLINE HEAT TREATMENT TEMPERATURE | REMARKS |
|---|---|---|---|---|---|---|---|---|---|---|---|---|---|---|---|
| | C | Si | Mn | P | S | Al | Ti | B | N | Cr | V | °C | °C | °C | |
| D30 | 0.50 | 0.85 | 0.72 | 0.015 | 0.010 | 0.060 | 0.040 | 0.0037 | 0.0036 | - | 0.120 | 950 | 750 | 500 | COMPARATIVE EXAMPLE |
| D31 | 1.25 | 0.90 | 0.72 | 0.008 | 0.006 | 0.030 | 0.048 | 0.0039 | 0.0047 | - | - | 960 | 780 | 520 | |
| D32 | 1.05 | 1.20 | 0.85 | 0.027 | 0.019 | 0.027 | 0.190 | 0.0054 | 0.0037 | - | 0.250 | 1135 | 860 | 420 | |
| D33 | 0.95 | 1.30 | 0.70 | 0.015 | 0.005 | - | 0.035 | 0.0036 | 0.0015 | - | - | 1130 | 850 | 450 | |
| D34 | 0.88 | 0.90 | 0.72 | 0.008 | 0.006 | 0.030 | 0.048 | 0.0039 | 0.0047 | - | - | 1080 | 780 | 520 | |
| D35 | 0.90 | 0.90 | 0.80 | 0.009 | 0.007 | 0.042 | 0.010 | - | 0.0060 | 0.23 | 0.210 | 980 | 735 | 520 | |
| D36 | 0.90 | 0.90 | 0.80 | 0.009 | 0.007 | 0.042 | 0.010 | - | 0.0060 | 0.23 | 0.210 | 980 | 880 | 520 | |
| D37 | 0.92 | 0.24 | 0.72 | 0.012 | 0.000 | 0.033 | - | 0.0040 | 0.0025 | 0.15 | - | 1000 | 790 | 550 | |
| D38 | 0.95 | 1.30 | 0.20 | 0.015 | 0.005 | - | 0.035 | 0.0036 | 0.0035 | - | - | 1000 | 785 | 550 | |

| | | | | | | | | | | | | | | | |
|---|---|---|---|---|---|---|---|---|---|---|---|---|---|---|---|
| UNDERLINED VALUE IS OUT OF RANGE OF PRESENT INVENTION | | | | | | | | | | | | | | | |

**[Table 4-1]**

| No | AVERAGE PBS | NUMBER DENSITY OF COARSE PB | TENSILE STRENGTH AT -40°C | ELONGATION AT -40°C | CHARPY IMPACT VALUE AT -40°C | CHARPY IMPACT VALUE AT ROOM TEMPERATURE | REMARKS |
|---|---|---|---|---|---|---|---|
| | *µ*m | | MPa | % | J | J | |
| D1 | 15 | 0 | 1201 | 18.0 | 15.0 | 25.0 | |
| D2 | 18 | 0 | 1265 | 17.8 | 14.7 | 24.0 | |
| D3 | 19 | 0 | 1295 | 17.1 | 14.0 | 23.9 | |
| D4 | 18 | 0 | 1380 | 16.8 | 13.0 | 23.4 | |
| D5 | 15 | 0 | 1390 | 16.6 | 13.2 | 23.0 | |
| D6 | 16 | 0 | 1430 | 16.2 | 13.8 | 23.0 | |
| D7 | 17 | 0 | 1410 | 16.3 | 13.5 | 22.5 | |
| D8 | 15 | 0 | 1490 | 15.9 | 13.6 | 21.0 | |
| D9 | 18 | 0 | 1460 | 15.6 | 14.0 | 22.0 | EXAMPLE |
| D10 | 20 | 0 | 1530 | 15.5 | 13.2 | 22.0 | |
| D11 | 19 | 0 | 1540 | 14.8 | 13.6 | 21.5 | |
| D12 | 18 | 0 | 1530 | 14.5 | 13.0 | 21.0 | |
| D13 | 20 | 20 | 1540 | 13.4 | 13.2 | 20.3 | |
| D14 | 23 | 18 | 1580 | 13.1 | 13.0 | 20.0 | |
| D15 | 22 | 0 | 1530 | 13.7 | 13.0 | 21.0 | |
| D16 | 23 | 0 | 1542 | 13.5 | 13.0 | 20.0 | |

**[Table 4-2]**

| No | AVERAGE PBS | NUMBER DENSITY OF COARSE PB | TENSILE STRENGTH AT -40°C | ELONGATION AT -40°C | CHARPY IMPACT VALUE AT -40°C | CHARPY IMPACT VALUE AT ROOM TEMPERATURE | REMARKS |
|---|---|---|---|---|---|---|---|
| | *µ*m | | MPa | % | J | J | |
| D17 | 28 | 44 | 1100 | 9.7 | 10.1 | 17.0 | COMPARATIVE EXAMPLE |
| D18 | 27 | 51 | 1210 | 9.5 | 10.0 | 15.0 | |
| D19 | 28 | 50 | 1230 | 9.2 | 9.5 | 16.0 | |
| D20 | 30 | 79 | 1255 | 8.7 | 9.0 | 16.0 | |
| D21 | 35 | 120 | 1280 | 8.6 | 8.6 | 15.3 | |
| D22 | 38 | 60 | 1310 | 8.0 | 8.5 | 15.1 | |
| D23 | 40 | 140 | 1420 | 7.0 | 7.0 | 15.1 | |
| D24 | 44 | 160 | 1400 | 7.5 | 7.5 | 14.7 | |
| D25 | 48 | 180 | 1480 | 6.0 | 7.2 | 14.6 | |
| D26 | 34 | 120 | 1580 | 5.4 | 7.0 | 14.3 | |
| D27 | 42 | 100 | 1525 | 5.6 | 6.9 | 15.0 | |
| D28 | 35 | 170 | 1540 | 5.4 | 6.5 | 14.1 | |
| D29 | 45 | 160 | 1570 | 5.4 | 6.0 | 14.0 | |

| No | PBS | NUMBER DENSITY OF COARSE PB | TENSILE STRENGTH AT -40°C | ELONGATION AT -40°C | CHARPY IMPACT VALUE AT -40°C | CHARPY IMPACT VALUE AT ROOM TEMPERATURE | REMARKS |
|---|---|---|---|---|---|---|---|
| | *µ*m | | MPa | % | J | J | |
| D30 | 21 | 20 | 1010 | 11 | 18.2 | 22.0 | COMPARATIVE EXAMPLE |
| D31 | 23 | 23 | 1590 | 5.1 | 3.0 | 9.0 | |
| D32 | 41 | 40 | 1310 | 6.3 | 6.2 | 14.0 | |
| D33 | 39 | 60 | 1300 | 6.9 | 6.0 | 14.3 | |
| D34 | 25 | 56 | 1375 | 6.2 | 8.5 | 14.0 | |
| D35 | 30 | 65 | 1250 | 5.1 | 7.8 | 13.0 | |
| D36 | 45 | 70 | 1385 | 9.2 | 9.8 | 15.2 | |
| D37 | 15 | 0 | 1380 | 3 | 4.2 | 9.5 | |
| D38 | 39 | 52 | 1490 | 4.9 | 5.3 | 13.2 | |

| | | | | | | | |
|---|---|---|---|---|---|---|---|
| UNDERLINED VALUE IS OUT OF RANGE OF PRESENT INVENTION | | | | | | | |

No. D1 to D16 of the Table 3 were examples satisfying the condition according to the present invention. On the other hand, No. D17 to D38 of the Table 4 were comparative examples which did not satisfy the conditions according to the present invention. Although the grain size of the pearlite block and the number density of the coarse PB of the example were controlled to the adequate level, the grain size of the pearlite block and the number density of the coarse PB of the comparative example were out of the range defined by the present invention. The examples demonstrated more excellent low-temperature strength, low-temperature toughness, and room-temperature toughness as compared with the comparative examples.

Figure 7A shows SEM picture of the pearlite block of the example and Figure 7B shows SEM picture of the pearlite block of the comparative example. It could be found from the SEM pictures that the grain size of the pearlite block of the example was clearly different from that of the comparative example.

Figure 8 shows a relationship between the grain size of the pearlite block (µm) and the impact value based on the impact value shown in Table 4. It could be found from the Figure 8 that the impact value of the example (PBS: 15 to 23µm) was higher than the impact value of the comparative example (PBS: 30 to 45µm) in both of room temperature and -40°C.

Figure 9A and Figure 9B show SEM observation result of the fracture surface of the charpy impact test piece of the example and comparative example. Figure 9A shows fracture facet of the example and Figure 9B shows fracture facet of the comparative example. The fracture facet of the example was finer than the fracture facet of the comparative example. This indicates that the example had more excellent toughness than the comparative example. In view of the point, the effect of refining PBS could be found.

Accordingly, it was found that the toughness of the example was higher than the toughness of the comparative example at both of room temperature and the environment of -40°C, to which the wire rod was exposed when the wire rod was used as additional PC of LNG tank.

### [Industrial Applicability]

According to the present invention, a wire rod for PC steel stranded wire which is used as tendon of PC dike of PC-type LNG tank and which has more excellent elongation at about -40°C as compared with the conventional material can be provided by reducing grain size of pearlite block. Therefore, the present invention contributes to enhancing reliability of the PC steel stranded wire, which is a member constructing equipments concerning LNG tank which is much in demand these days, under low-temperature usage environment, and thus, the present invention has significant industrial applicability.

### [Brief Description of the Reference Symbols]

1: wire rod
2: 2mm U-notch charpy impact test piece
3: 2mm U-notch

## Claims

1. A wire rod, wherein
the chemical composition consists of, in terms of mass%:
C: 0.60 to 1.20%;
Si: 0.80 to 1.30%;
Mn: 0.30 to 0.90%;
P: 0.020% or less;
S: 0.020% or less;
N: 0.0025 to 0.0060%;
Cr: 0 to 1.00%;
V: 0 to 0.800%;
one or more selected from the group consisting of
Al: 0.005 to 0.100%,
Ti: 0.003 to 0.050%, and
B: 0.0005 to 0.0040%; and
the remainder including Fe and impurity,
wherein an average value of a grain size of a pearlite block in a cross section perpendicular to a wire rod axial direction is 23 µm or less, and
wherein a number density of the pearlite blocks having 40 µm or more of the grain size in the cross section perpendicular to the wire rod axial direction is 0 to 20 pieces/mm².

2. The wire rod according to claim 1, wherein
the chemical composition includes one or more selected from the group consisting of, in terms of mass%:
Cr: 0.10 to 1.00%, and
V: 0.005 to 0.800%.

3. The wire rod according to claim 1, wherein
the chemical composition includes, in terms of mass%:
C: 0.70 to 0.90%;
Mn: 0.60 to 0.90%; and
V: 0 to 0.500%.

4. The wire rod according to claim 3, wherein
the chemical composition includes one or more selected from the group consisting of, in terms of mass%:
Cr: 0.50 to 1.00%, and
V: 0.300 to 0.500%.

5. The wire rod according to any one of claims 1 to 4, wherein
the chemical composition includes one or more selected from the group consisting of, in terms of mass%,
Al: 0.020 to 0.050%, and
Ti: 0.020 to 0.040%.

6. A method for manufacturing the wire rod, the method comprising:
heating a steel piece having the chemical composition according to claim 3 or 4 to a rough-rolling temperature of 950 to 1040°C and rough-rolling;
finish-wire-rolling at a finish-rolling temperature of 750 to 950°C;
then, coiling at a coiling temperature of 730 to 840°C; and thereafter,
air blast cooling to a temperature range of 5 to 35°C with a cooling rate of 15°C/sec or more,
wherein the finish-rolling temperature and a strain rate in the finish-wire-rolling satisfy an expression A, $13.7 \leq {log}_{10} \left\{\left(dε / dt\right) \times exp ( 63800 / \left(1.98 \times \left(T + 273.15\right)\right)\right\} \leq 16.5$ and
wherein dε / dt expresses the strain rate in the finish-wire-rolling in terms of s⁻¹ and T expresses the finish-rolling temperature in terms of °C.

## Patentansprüche

1. Ein Walzdraht, wobei
die chemische Zusammensetzung, ausgedrückt in Massen-%, aus
C: 0,60 bis 1,20%;
Si: 0,80 bis 1,30%;
Mn: 0,30 bis 0,90%;
P: 0,020% oder weniger;
S: 0,020% oder weniger;
N: 0,0025 bis 0,0060%;
Cr: 0 bis 1,00%;
V: 0 bis 0,800%;
einem oder mehreren, ausgewählt aus der Gruppe bestehend aus
Al: 0,005 bis 0,100%,
Ti: 0,003 bis 0,050% und
B: 0,0005 bis 0,0040%, besteht; und
der Rest Fe und Verunreinigung beinhaltet,
wobei ein Mittelwert einer Korngröße eines Perlitblocks in einem Querschnitt senkrecht zu einer Axialrichtung eines Walzdrahts 23 µm oder weniger beträgt und wobei eine Zahlendichte der Perlitblöcke mit einer Korngröße von 40 µm oder mehr im Querschnitt senkrecht zur Axialrichtung des Walzdrahts 0 bis 20 Stück/mm² beträgt.

2. Der Walzdraht nach Anspruch 1, wobei
die chemische Zusammensetzung, ausgedrückt in Massen-%, eines oder mehrere, ausgewählt aus der Gruppe bestehend aus:
Cr: 0,10 bis 1,00% und
V: 0,005 bis 0,800%, beinhaltet.

3. Der Walzdraht nach Anspruch 1, wobei
die chemische Zusammensetzung, ausgedrückt in Massen-%:
C: 0,70 bis 0,90%;
Mn: 0,60 bis 0,90%; und
V: 0 bis 0,500% beinhaltet.

4. Der Walzdraht nach Anspruch 3, wobei
die chemische Zusammensetzung, ausgedrückt in Massen-%, eines oder mehrere, ausgewählt aus der Gruppe bestehend aus:
Cr: 0,50 bis 1,00% und
V: 0,300 bis 0,500%, beinhaltet.

5. Der Walzdraht nach einem der Ansprüche 1 bis 4, wobei die chemische Zusammensetzung, ausgedrückt in Massen-%, eines oder mehrere, ausgewählt aus der Gruppe bestehend aus
Al: 0,020 bis 0,050% und
Ti: 0,020 bis 0,040%, beinhaltet.

6. Ein Verfahren zur Herstellung des Walzdrahts, wobei das Verfahren umfasst:
Erwärmen eines Stahlstücks mit der chemischen Zusammensetzung nach Anspruch 3 oder 4 auf eine Vorwalztemperatur von 950 bis 1040°C und Vorwalzen;
Drahtfertigwalzen bei einer Fertigwalztemperatur von 750 bis 950°C;
dann Aufwickeln bei einer Aufwickeltemperatur von 730 bis 840°C; und danach Luftstromkühlen auf einen Temperaturbereich von 5 bis 35°C mit einer Abkühlgeschwindigkeit von 15°C/s oder mehr,
wobei die Fertigwalztemperatur und eine Dehnungsrate beim Drahtfertigwalzen einen Ausdruck A erfüllen, $13,7 \leq {log}_{10} \left\{\left(dε / dt\right) \times exp ( 63800 / \left(1,98 \times \left(T + 273,15\right)\right)\right\} \leq 16,5$ und
wobei dε / dt die Dehnungsrate beim Drahtfertigwalzen in s⁻¹ ausdrückt und T die Fertigwalztemperatur in °C ausdrückt.

## Revendications

1. Fil machine, dans lequel
la composition chimique est constituée, en termes de % en masse, de :
C: 0,60 à 1,20 % ;
Si: 0,80 à 1,30 % ;
Mn : 0,30 à 0,90 % ;
P : 0,020 % ou moins ;
S : 0,020 % ou moins ;
N : 0,0025 à 0,0060 % ;
Cr: 0 à 1,00 % ;
V : 0 à 0,800 % ;
un ou plusieurs choisis dans le groupe constitué de Al : 0,005 à 0,100 %,
Ti : 0,003 à 0,050 %, et
B : 0,0005 à 0,0040 % ; et
le reste incluant du Fe et des impuretés,
dans lequel une valeur moyenne d'une taille de grains d'un bloc de perlite dans une coupe transversale perpendiculaire à la direction axiale du fil machine est de 23 µm ou moins, et
dans lequel une densité en nombre des blocs de perlite ayant 40 µm ou plus de la taille de grains dans la coupe transversale perpendiculaire à la direction axiale du fil machine va de 0 à 20 pièces/mm².

2. Fil machine selon la revendication 1, dans lequel
la composition chimique inclut un ou plusieurs choisis dans le groupe constitué, en termes de % en masse, de :
Cr: 0,10 à 1,00 %, et
V : 0,005 à 0,800 %.

3. Fil machine selon la revendication 1, dans lequel la composition chimique inclut, en termes de % en masse :
C : 0,70 à 0,90 % ;
Mn : 0,60 à 0,90 % ; et
V : 0 à 0,500 %.

4. Fil machine selon la revendication 3, dans lequel
la composition chimique inclut un ou plusieurs choisis dans le groupe constitué, en termes de % en masse, de :
Cr : 0,50 à 1,00 %, et
V : 0,300 à 0,500 %.

5. Fil machine selon l'une quelconque des revendications 1 à 4, dans lequel
la composition chimique inclut un ou plusieurs choisis dans le groupe constitué, en termes de % en masse, de,
Al : 0,020 à 0,050 %, et
Ti : 0,020 à 0,040 %.

6. Procédé de fabrication du fil machine, le procédé comprenant :
le chauffage d'une pièce d'acier ayant la composition chimique selon la revendication 3 ou 4 à une température de laminage brut de 950 à 1040 °C et le laminage brut ;
le laminage de finition de fil à une température de laminage de finition de 750 à 950 °C ;
puis, le bobinage à une température de bobinage de 730 à 840 °C ; et par la suite,
le refroidissement par jet d'air à une plage de température de 5 à 35 °C avec une vitesse de refroidissement de 15 °C/s ou plus,
dans lequel la température de laminage de finition et le taux de déformation au cours du laminage de finition de fil satisfont une expression A, $13,7 \leq {log}_{10} \left\{\left(dε / dt\right) \times exp ( 63800 / \left(1,98 \times \left(T + 273,15\right)\right)\right\} \leq 16,5$ et
dans lequel dε / dt exprime le taux de déformation au cours du laminage de finition de fil en termes de s⁻¹ et T exprime la température de laminage de finition en termes de °C.
